

Dec. 12, 1933.

I. C. W. MANN

1,938,707

PROCESS OR METHOD OF CASTING

Filed July 28, 1930



INVENTOR  
Ira C. W. Mann

ATTORNEYS

W. L. Mann, H. L. Mann, W. L. Mann & H. L. Mann

## UNITED STATES PATENT OFFICE

1,938,707

## PROCESS OR METHOD OF CASTING

Ira C. W. Mann, Lansing, Mich., assignor to Reo Motor Car Company, Lansing, Mich., a corporation of Michigan

Application July 28, 1930. Serial No. 471,325

1 Claim. (Cl. 22—204)

This invention relates to a cast metal plate having a pin of different material cast therein and to the process or method of casting the same.

5 The invention relates particularly to a cast iron punch plate having a steel pilot pin cast therein and to the method of making the same.

Heretofore it has been the custom to employ in connection with punch presses and the like, a 10 punch plate formed of cast iron or the like having formed thereon an integral cast projection or pin by means of which the plate is secured to the press. It has been found in practice, however, that cast iron pins or projections cast with 15 the plate when the same is made are apt to fracture and frequently do at the juncture of the pin with the plate.

It is therefore one of the important objects of my invention to provide a punch plate having 20 a steel pin secured thereto when the plate is cast, it being found that in structures of this kind all liability of fracture at the juncture of the plate and pin is eliminated.

The several objects and advantages of my invention together with the manner in which my improved method or process is practiced will be 25 made more apparent as this description proceeds, especially when considered in connection with the accompanying drawing, wherein

30 Figure 1 is a perspective view of a punch plate constructed in accordance with my invention and in accordance with my process;

Figure 2 is a vertical sectional view through a mold by means of which the plate is cast, and

35 Figure 3 is a top plan view of the core of the mold.

As seen from Figure 1, the punch plate 10 is cast with a pilot or pin 11, formed preferably of 40 steel and united with the plate 10 when the latter is cast.

By reference to Figures 2 and 3 the manner in which the punch plate 10 is cast will be made 45 more apparent. In this figure it will be noted that the mold consists of a drag section 12 and a cope section 13. The drag section of the mold is provided with the punch plate pattern recess or cavity 14. The drag section of the mold is 50 preferably rammed full of sand with the bottom side up, the sand being rammed around the punch plate pattern (not shown) which would then be in the bottom thereof. The drag section of the mold is then turned over placing the pattern on top.

The reference character 15 indicates the core 5 of the mold which as shown in Figure 3, is formed

of two sections 15'. The two halves of the core are recessed to accommodate the end of the pilot or pin 16 and after being placed together these two core halves are cemented together to thus hold the pilot or pin in place. The core is provided with a plurality of vertically extending apertures 17 arranged circumferentially around the pilot 16.

The core together with the pilot 16, is placed in the cope section of the mold and for locating the pilot with respect to the mold cavity during the time that sand is rammed into the cope section of the mold, the punch plate pattern which is still in the drag section of the mold is provided with an aperture 18, see the dotted line illustration of a portion of the punch plate pattern shown in Figure 2.

Therefore with the core in position and with the pilot 16 extending down into the aperture 18, sand is rammed around the core firmly to hold the core in the position shown. At the same time a riser (not shown) is inserted in the upper flask to provide the riser opening 19.

After the cope section has been rammed full of sand it is removed on the parting line, the pattern is taken out together with the member which formed the riser opening and an outlet is made communicating with the riser opening. Thereafter the cope section is again placed on the drag section of the mold whereupon the pilot or pin 16 will project down into the pattern recess or cavity 14. Thereafter a runner box 20 is placed on top of the cope section of the mold in position to surround the core 15. Also an over-flow basin 21 is placed at the side of the mold adjacent the riser and the molding apparatus is ready

for the pouring of the molten metal.

At this point it might be noted that the pilot or pin 16 is preferably made of cold-rolled steel and copper plated. In the first place, this prevents rusting of the pilot and the copper serves as a flux to insure an adequate union between the pilot and the cast iron of which the punch plate is formed.

The metal is then poured into the runner box 100 in sufficient quantities and fast enough to keep the runner box substantially completely full, thus creating a static head or pressure which acts to force the molten metal down through the circumferentially arranged apertures 17 and into 105 the mold cavity 14. After the mold cavity 14 is full, the metal overflows through the riser and flows into the over-flow basin 21.

In practice it has been found efficient to pour 110 into the mold a surplus of metal substantially

equal to the amount required to fill the pattern recess or cavity 14. This surplus of hot molten metal which flows through the apertures 17 and into the pattern recess heats the pilot or pin 16 substantially to a melting point which causes the pilot and the plate to unite. By reason of the fact that the pilot becomes thoroughly heated throughout its length, it does not cool quicker than or prior to the plate 10 so that there is no difference in the coefficient of expansion or contraction which would permit the pilot 16 to become loose with respect to the plate. Moreover, it is desirable, although not essential, that the end of the pilot 16 be provided with a circumferential groove or reduced portion 16' into which the molten metal will flow to provide a more adequate union between the parts. In practice it also has been found that by maintaining the pin heated throughout its length it will not chill and harden the cast iron and prevent machining.

When the cast article has become sufficiently chilled to be removed from the mold, the core 15 is obviously removed from the pilot 16.

25

Various modifications of the specific method herein described may suggest themselves to those skilled in this art and to this end reservation is made to make such changes as may come within the purview of the accompanying claim.

80

What I claim as my invention is:

Those steps in the method of integrating a steel pilot with a cast iron punch plate which consist in forming a cavity in a lower mold part, said cavity being of the size and shape of the punch desired, mounting a pilot in a core member with the end of the pilot projecting from the core member, mounting said core member in a second mold part, assembling said second mold part with the first mentioned mold part with the projecting end of the pilot disposed in the cavity in the first mentioned mold part, forming passages in the core member circumferentially of the pilot, and pouring molten casting metal into said cavity by way of said passages.

85

90

95

IRA C. W. MANN.

100

30

105

35

110

40

115

45

120

50

125

55

130

60

135

65

140

70

145